

March 7, 1933.

A. L. CLAPP

1,900,427

MANUFACTURE OF FIBROUS ARTICLES

Filed Dec. 20, 1927



Inventor:  
Albert L. Clapp,  
by  
Wright Brown, New York  
Attest:

## UNITED STATES PATENT OFFICE

ALBERT L. CLAPP, OF DANVERS, MASSACHUSETTS

## MANUFACTURE OF FIBROUS ARTICLES

Application filed December 20, 1927. Serial No. 241,436.

This invention relates to the manufacture of fibrous articles using paper pulp as a raw material and using papermaking machinery, so that such articles may be manufactured 5 rapidly and economically.

In manufacturing fibrous articles using paper pulp as a raw material, it has sometimes been the practice to mould the pulp in a free or lightly beaten condition under suction or pressure between foraminous moulds, then to remove the articles from the moulds and dry them. Articles thus produced are quite porous and of comparatively poor strength, doubtless because of the loose, random arrangement of the fibers resulting from moulding. If it be attempted to improve the characteristics of such articles by thoroughly beating the pulp or by incorporating filling or sizing materials into the pulp, it is found that the slow or beaten pulp or such filling materials tend to interfere with successful moulding, by plugging up the interstices of the foraminous moulds.

One of the objects of the present invention is to make possible the production of fibrous articles in which the fibers exist in the compacted, interfeltd condition resulting from manufacture on papermaking machinery. The method of the present invention involves running the paper pulp off into a web on a paper machine, and then while the web is still wet, preferably as it comes off the wet end of the machine, forming it into articles of the desired shape.

A method such as described is particularly advantageous when it is desired to use filling and/or sizing materials in the manufacture of fibrous products, as such materials may be incorporated into the pulp in the beater engine, and the pulp run off into a web on the wet end of a paper machine without difficulty, even if such material would cause difficulty on the dry end of the machine. Any waste material resulting from cutting or moulding the wet web may be returned to the beater engine and easily disintegrated and conditioned for the production of other web material. My method may, for instance, be employed to advantage 50 when thermoplastic waterproofing materials

in finely divided or dispersed condition are incorporated into the pulp, as any waste resulting from the production of articles from a wet web prepared from the pulp may be easily conditioned for web formation. If, 55 on the other hand, a web containing such thermoplastic material were once dried and the material fused on the fibers, it would be quite difficult to disintegrate the web into its component fibers and to condition them 60 for satisfactory web formation. My method also permits the use of high proportions of thermoplastic material with the pulp in the beater furnish, as the beater furnish may be run off into a web on the wet end of a paper 65 machine without difficulty, whereas sticking and breaking of the web would be likely to take place if it were attempted to run such a web over the dry end of the machine.

The wet web may be cut or moulded into 70 various articles. For instance, if a wet web of the proper caliper and containing sufficient waterproofing material for the manufacture of roofing products is prepared, it may be cut up into roofing shingles of the desired shape, or moulded into roofing tile, any 75 waste resulting from cutting or moulding being returned to the beater engine. The shingles or tile may then be dried at a temperature sufficient to cause a fusion of the 80 thermoplastic waterproofing material contained therein and thus to ensure the encasing of the fibers and the filling of the pores and interstices of the web with such material. If desired, drying may be effected between heated dies under pressure to effect a 85 compacting of the product.

A web of pulp comes off the wet end of the paper machine in a sufficiently dewatered condition to be self-sustaining, but it is still 90 of low strength, so that when it is desired to mould articles therefrom, moulding must be effected gradually and under light pressure, as otherwise the web would be liable to break. Furthermore, the moulds must also be designed to allow moulding without breaking of the web. To this end, the moulds which are employed are preferably lined with a soft or yieldable material such as felt, 95 which serves to back up the wet web while 100

it is being moulded. After moulding, the articles are removed from the moulds and dried. Inasmuch as light, yielding pressure is applied during moulding, the articles may 5 have substantially the same water content as the wet web before moulding.

If articles are moulded from a wet web of ordinary paper pulp, such as kraft, sulphite, or ground-wood pulp, and then dried, 10 they generally tend to warp badly and lose their shapes. I have found that this difficulty may be overcome by incorporating certain materials in suitable proportion into the paper pulp from which the wet web is 15 formed. Thus, if a certain amount of non-hydratable material such as asbestos fiber is incorporated into the pulp, the wet web formed from such pulp may be moulded into articles which have practically no tendency 20 to warp upon drying, even when the pulp is beaten out sufficiently to yield a product of optimum density and strength. The amount of asbestos fiber necessary for this purpose will vary, depending upon the character of 25 the pulp used as a raw material and the shape or other characteristics of the articles, some pulp yielding articles having greater tendencies to warp than others. Thus, articles made from kraft pulp have a greater tendency 30 to warp than similar articles made of sulphite pulp, and those made of the latter pulp have a greater tendency to warp than those made of ground-wood pulp. I have further found that if sufficient amount of 35 thermoplastic waterproofing material is incorporated into the pulp, it will also inhibit warping of articles moulded from a web prepared from such pulp.

Various non-warping pulp compositions 40 may be employed in the practice of my invention. For instance, I may employ a composition comprising 90 parts ground-wood pulp and 10 parts asbestos fiber, or one comprising 50 parts of kraft pulp and 50 parts 45 asbestos fiber, or another comprising 20 parts sulphite pulp, 50 parts ground-wood pulp, and 30 parts asbestos fiber. Filling materials such as ground-asbestos, lime, magnesium oxide, clay, cellite, infusorial earth, 50 and wood flour, when incorporated into the pulp also tend to prevent warping of articles made from the sheeted pulp, but I prefer to use asbestos fiber along with such materials, for when such materials alone are used 55 in suitable quantity to prevent warping, a product of optimum strength is not obtained. In lieu of, or in addition to asbestos and/or other filling materials, I may incorporate suitable thermoplastic waterproofing materials 60 into the pulp and produce a precipitate therein to fix such waterproofing materials on the fibers. For instance, I may charge the beater engine with 60 parts of pulp and 40 to 80 parts of thermoplastic material in 65 pulverized condition or dispersed in a suit-

able dispersing agent, e. g., soap or sodium silicate solution. Ten parts of 40° Baumé sodium silicate may then be added, together with 5 parts of alum, to produce a flocculent precipitate of aluminum silicate, which 70 serves to carry down and fix the thermoplastic material on the pulp. The beater furnish may then be run off into a web on the wet end of a paper machine, and the wet web then moulded into articles which when dried 75 have no tendency to warp. Drying is preferably performed below the softening point of the thermoplastic material, as otherwise the articles tend to sag and become deformed, owing to their high content of thermoplastic material. This tendency to sag may be overcome by substituting asbestos for part of the thermoplastic material. For instance, if a beater furnish comprising 70 parts of pulp, 20 parts of asbestos, and 20 parts of waterproofing material is run off into a wet web moulded into articles, such articles may be dried at a temperature sufficiently high to cause fusion of the thermoplastic material 80 therein without danger of sagging. If the wet web is cut into flat articles, such as roofing shingles, however, the proportion of thermoplastic waterproofing material may run as high as from 40% to 80% of the total dry materials added to the beater, and drying may be effected while the articles are supported in a flat condition, at a temperature 85 sufficiently high to cause the fusion of the thermoplastic material therein.

Various thermoplastic materials may be 90 employed to prevent warping and to waterproof the product, depending upon the characteristics desired in the final product. For instance, where discoloration of the product is to be avoided, waxes such as paraffin, montan, or carnauba, together with free rosin, may be employed. Where discoloration of the product is immaterial, as in the manufacture of roofing products, bitumens, or asphalts, e. g., those having a melting point 95 ranging from 200° to 400° F. may be employed.

Another object of the present invention is 100 to provide a method of and means for continuously moulding articles of the desired shape from the wet web of pulp as it comes off the wet end of the paper machine. To this end, the wet web is passed between one or more pairs of endless series of moving moulds, which gradually close and act to mould successively portions of the web into articles of the desired shape, then sever the articles from the web, then open, whereupon the articles are successively removed 105 from the moulds, and then return to initial position. Preferably, the articles are removed onto an endless conveyor belt which serves to carry them in continuous fashion 110 through a drying chamber.

The present invention will now be de- 115

scribed in connection with the moulding of pie plates, it being understood that this is illustrative, many other articles, such as pans or other containers, roofing tiles, etc., being 5 mouldable in accordance with the present invention. Where asbestos or fillers such as lime are incorporated into the pulp to prevent warping and articles such as pie plates are being made, I may advantageously treat 10 the wet web or the articles made therefrom with sodium silicate solution, as the treatment yields a product which is waterproof, greaseproof, and fireproof after drying. Preferably, this treatment is effected after 15 the articles are formed, so as to avoid sticking and tendency of the web to break during the forming of the articles.

On the accompanying drawing,

Figure 1 represents somewhat diagrammatically and conventionally an assembly of 20 means for manufacturing pie plates in accordance with the present invention.

Figure 2 represents a side view, partly in 25 section, of a pair of endless series of moulds operating on a wet web of pulp as it comes from the web-forming mechanism.

Figure 3 represents a section through a pair of mould members for forming the plates.

Figure 4 shows in perspective a portion of 30 the web of pulp after moulding has been completed.

Figure 5 is a perspective view of the moulded plate.

Referring in detail, first, to Figure 1 of the drawing, A represents as a whole the web-forming mechanism, which may be of any suitable type, that shown in the drawings being the wet end of a cylinder papermaking 40 machine. The machine comprises a vat 1, into which the paper pulp is introduced at the usual papermaking consistency.

Rotating partially submerged in the pulp contained in the vat is a cylinder mould 2, 45 on which a web of pulp is continuously deposited, the web being picked up from the unsubmerged portion of the mould by a traveling felt 3 maintained in contact with the cylinder mould by a couch roll 4. The 50 felt carries the web under an upper felt 5, where it is sufficiently dewatered to withstand passing between press rolls without being disintegrated, whence it carries the web successively between pairs of press rolls 6 and 55 7. The web now has a water content of about 60% to 70%, and while it is still liable to break, it is sufficiently strong to be self-sustaining, and as shown passes from the paper machine between one or more pairs of 60 endless mould carriers C, arranged transversely on the sheet.

As shown in Figure 2, one carrier of a pair is arranged immediately above the other carrier, both carriers gradually converging 65 in the direction of travel of the paper web

W as it passes therebetween from the paper machine. The upper carrier comprises an endless chain 9 mounted on a pair of sprockets 10, 10a, either one of which may be driven and thus serve to drive the chain. An endless series of male mould members 11, designed to mould pie plates, are carried at regularly-spaced intervals by the links of the chain. The lower carrier is of a construction similar to the upper one, except that it 70 carries an endless series of female mould members 13. Preferably, the upper stretch of the lower carrier is kept from sagging by a supporting platform 14, over which it passes. Both carriers are driven at the same rate of speed in the direction of travel of the web, and the mould members are mounted to cooperate with one another as they come together, there being sufficient slack in the 75 chains to permit proper alignment of the moulds. When the carriers have passed around the sprockets 10a into substantially horizontal position, a male mould 11 descends to press the web of pulp slightly into the female mould 13. As the carriers proceed, 80 the moulds gradually come together and close, thus pressing portions of the web downwardly out of the plane of the remainder of the web into plate form. The pressure 85 exerted is quite gradual and light, so that there is little tendency to break or disintegrate the web. Preferably, as shown in Figure 3, each of the mould members is lined with a layer of soft cloth or felt 17, so that any excess pressure or shocks will be absorbed.

As the forming of the plate is being completed, an annular knife 18 fixed to the marginal portion 19 of the upper mould member cuts through the web against the lower mould member and severs the formed plate thereon. The lower mould member with the plate contained therein proceeds around the sprocket 10, the plate generally tending to fall out by gravity as the mould member is inverted. If in any case there is a tendency for the plate to stick to the mould, means are preferably provided for removing it. Such means, for instance, may consist of an air blast delivered against the bottom of the 110 mouldled plate. As shown on the drawing, the lower sprocket shaft 15 is made hollow, so that air may be delivered thereinto from a supply pipe 20. Communicating with the interior of the shaft 15 and arranged radially thereof, is a blast pipe 21, which delivers a blast of air against the bottom of a formed plate, when a port 22 formed through the bottom of the mould member 13 to the felt lining comes into registry therewith. Preferably, as shown, a conveyor belt 23 is arranged to receive the plates as they fall from the successive moulds, the belt carrying the plates through a heating chamber 24, where 115 in they are dried and then delivered onto a 120 conveyor belt 25.

table 25, from which they may be removed for packing and shipment.

As illustrated in Figure 4, three pairs of series of moulds operate on a single web of pulp as it comes from the web-forming mechanism. A greater or less number might of course be used if desired. If desired, the wet web may be slit longitudinally between the several series of moulds before being moulded, as indicated by the dotted lines. The web material remaining after the plates have been cut therefrom may be returned to the beater while still in wet condition, where disintegration into pulp may be easily effected, or, as shown in Figure 1, may be wound up into a roll R before being returned to the beater. Articles may be moulded and cut in the manner just described, from single or multi-ply webs.

I am aware of the fact that it has been proposed to dampen or wet previously dried paper prior to moulding articles therefrom, but my invention departs considerably from such practice, for a web coming off the wet end of a paper machine is in a quite different condition from a web which has been dried. In such latter case, the web is in a compact, shrunk condition, so that moulding must take place between metal moulds under considerable pressure. Such latter procedure is furthermore much more expensive, as it involves the expense incident to drying and re-wetting the paper, and it requires much more power to disintegrate and beat up the resulting waste paper.

I do not herein claim per se the treatment of a fibrous web or articles containing asbestos or fillers such as lime, with an aqueous solution of sodium silicate, or the product resulting therefrom, as this is disclosed and claimed in my application, Serial No. 94,329, filed March 12, 1926.

Having thus described certain embodiments of this invention, it is obvious to those skilled in the art that various changes or modifications might be made therein without departing from the spirit or scope of invention as defined by the appended claims.

What I claim is:

1. Steps in the manufacture of pulp articles, which comprise preparing an aqueous pulp suspension containing sufficient non-hydratable material to form a non-warping composition, interfelting the pulp into a web on a paper machine, removing the web while wet from the machine, forming articles of the desired shape from the wet web, impregnating the articles with sodium silicate solution, and drying the treated articles.
2. Steps in the manufacture of pulp articles, which comprise interfelting the pulp into a continuous web on a paper machine, continuously removing the web from the wet end of the machine, progressively moulding portions of the web gradually and under

light pressure out of the plane of the web into articles of the desired shape, and severing the moulded articles from the web.

3. Steps in the manufacture of pulp articles, which comprise interfelting the pulp into a continuous web on a paper machine, continuously removing the web from the wet end of the machine, progressively moulding portions of the web gradually and under light pressure out of the plane of the web into articles of the desired shape, severing the moulded articles from the web, and drying the moulded articles.

4. Steps in the manufacture of pulp articles, which comprise incorporating sufficient non-hydratable material into cellulose pulp to form a non-warping composition, interfelting the composition into a web on a paper machine, removing the web while wet from the machine, moulding articles of the desired shape from the wet web and out of the plane of the web, severing the moulded articles from the wet web, and drying the wet articles.

5. Steps in the manufacture of pulp articles, which comprise incorporating sufficient asbestos into cellulose pulp to form a non-warping composition, interfelting the composition into a web on a paper machine, removing the web while wet from the machine, moulding articles of the desired shape from the wet web and out of the plane of the web, severing the moulded articles from the wet web and drying the wet articles.

In testimony whereof I have affixed my signature.

ALBERT L. CLAPP.

105

110

115

120

125

130